

Aug. 21, 1928.

1,681,353

M. LÉVY

PROCESS OF FORMING ROADS AND THE LIKE

Original Filed Nov. 2, 1922



M. Levy  
INVENTOR  
By: Marks & Clark  
Atty's.

Patented Aug. 21, 1928.

1,681,353

# UNITED STATES PATENT OFFICE.

MARCEL LÉVY, OF GENEVA, SWITZERLAND, ASSIGNOR TO "PRODOR" FABRIQUE DE PRODUITS ORGANIQUES S. A., OF GENEVA, SWITZERLAND.

## PROCESS OF FORMING ROADS AND THE LIKE.

Original application filed November 2, 1922, Serial No. 598,651, and in Great Britain January 3, 1922.

Divided and this application filed July 23, 1924. Serial No. 727,574.

In my application Serial No. 598,651 filed 55  
2nd November, 1922, I have dealt with the  
manufacture of concretes from a special hard  
pitch and a graded filling.

5 The object of the present invention is to  
provide a method of forming a paving or  
roadway employing such concrete.

The aforesaid concrete has nothing in common 10  
with tar products which are used for  
coating or paving roads, pavements or the  
like because these products must usually be  
comparatively soft and elastic. The new  
concrete cannot be so employed satisfactorily  
because it may have a liability to crack under  
15 the impact of steel tyres or horses' hoofs.

I have found, however, that this pitch concrete 20  
may be successfully used in the manufacture  
of road surfaces and the like if it is  
covered by a thin coating of some more  
plastic body which deadens the shocks, such  
25 as a body for example as asphalt.

Thus, the pitch concrete as indicated in  
application No. 598,651 may be used on roads  
or pavements in place of cement concretes  
25 which in certain cases are coated with a layer  
of asphalt.

The reason why the pitch concrete used 30  
in the present invention may replace cement  
concretes for the purpose specified is that  
it has mechanical properties substantially  
similar to cement concrete, that is to say  
35 it is hard, and non-plastic, has a crushing  
strength of at least about 4,000 to 5,000 lbs.  
per square inch, has a tensile strength when  
tested in the manner of testing cement  
concretes, that is to say without the large  
40 particles of the aggregate of at least about 400  
to 500 lbs. per square inch, and has a sub-  
stantial resistance to abrasion or wear.

40 With such pitch concrete according to the  
invention, I find that only a thin layer of  
asphalt is necessary. The asphalt or like  
plastic body is not relied on to give strength  
but merely to assist in minimizing the effect  
45 of shocks. It amalgamates with or welds  
solidly to the pitch concrete base and there  
is little tendency for it to flow from the  
centre to the sides of the road, the required  
covering being quite thin.

50 This invention therefore consists in a  
method of manufacturing a road, pavement  
or the like which comprises the provision of  
a pitch concrete made according to copending  
application No. 598,651 and a relatively

thin coating of a resilient or elastic substance, for example, asphalt. Tar or a mixture of pitch and tar may be used in place of asphalt.

The accompanying drawing shows a section 60  
of a road constructed according to one form  
of the present invention.

In the drawing, the roadway is indicated  
by the letter *a*. Above this, there is a stone  
foundation *b* carrying a mixture, marked *c*,  
of hard pitch, broken stone, sand and powder,  
reference to which is given in more detail  
below, the whole being covered by an asphalt  
surface *d*.

Such a paving may for example be constructed 70  
in the following manner:

The new concrete is first poured on to the  
surface to be covered and then a resilient and  
elastic material is poured on to the concrete  
sub-structure.

Paving slabs may also be formed from 75  
the new concrete, of which the surface is  
coated with a layer of resilient and elastic  
material.

Such an example will now be given:

The following substances are mixed together  
while being heated:

450 kgs. gas pitch, mineral oil pitch or any  
other pitch of inferior and cheap quality,  
which remains hard in water at 70° C. (In  
order to determine the hardness, a thin piece 85  
of this pitch is placed in the hot water and  
heated for some minutes. The pitch should  
remain quite hard at the temperature in  
question and should not be flexible nor show  
an indentation on pressure with the thumb 90  
nail.);

3500 kgs. of broken limestone or gravel;

1500 kgs. ordinary sand;

700 kgs. pulverized limestone.

The hot mixture is spread out on a stone 95  
surface or the floor in order to obtain a  
layer of 5-15 cm. thickness. As soon as  
the mass has set and while still hot it is  
coated with a layer of asphalt 5-20 mm.  
thick. The road or paving obtained in this 100  
manner forms after setting a single block as  
the asphalt layer effectively and solidly ad-  
heres to the sub-structure of pitch concrete.  
As will be seen from the foregoing the pres-  
ent process differs from the known processes 105  
by reason of the fact that a solid and strong  
concrete is first produced, which however is  
too hard to withstand without damage the

shocks on pavements or roads due to traffic and horses' hoofs, for which reason a layer of asphalt is poured thereon so that both layers intimately combine with one another and form a solid entirety. If a piece of the new concrete coated with asphalt is broken off with a hammer, then the asphalt layer remains firmly attached to the concrete and the fracture is similar to that which would be formed were the whole mass entirely homogeneous.

In order to facilitate the combination of an old pitch concrete with a new one the surface of the old concrete may be coated with a varnish or simply with tar or a thin layer of soft asphalt may be poured between the old and the new concrete while the latter is still hot and viscous. This can be done in the following manner:—

The new still viscous and soft layer of concrete is separated from the old layer by a trowel and asphalt is poured into the small intervening space. In this manner an effective combination is obtained between the two layers while the connecting layer is at the same time also elastic.

The new concrete covered with a plastic layer may also be used for indoor floors.

Having now described my invention, what I claim as new and desire to secure by Letters Patent is:—

1. The method of laying a roadway which

comprises forming a substratum of a pitch concrete which is hard, non-plastic and has a crushing strength of at least about 4,000 to 5,000 lbs. per square inch and tensile strength when the large aggregate is not present of about 400 to 500 lbs. per square inch and substantially retains these properties under temperature conditions of use by first mixing said pitch concrete by incorporating into hard pitch under the action of heat a graded aggregate and filling material, laying this mixed pitch concrete as a substratum and covering this substratum with a thin coating of a plastic substance which solidly adheres thereto.

2. A method as claimed in claim 1, in which the plastic substance is plastic asphaltum-like matter.

3. Roadway blocks made of pitch concrete having a crushing strength of at least about 4,000 to 5,000 lbs. per square inch and tensile strength when the large aggregate is not present of about 400 to 500 lbs. per square inch and substantially retains these properties under temperature conditions of use, containing a graded filling material and coated at least on one surface with a thin coating of a plastic asphaltum-like substance which solidly adheres thereto.

In testimony whereof I have signed my name to this specification.

MARCEL LÉVY.